

Patented Nov. 28, 1922.

## UNITED STATES PATENT OFFICE.

FREDERICK L. WHITE, OF LAKEWOOD, OHIO, ASSIGNOR TO JOSEPH A. WILLIAMS, OF CLEVELAND, OHIO.

## ALLOY FOR ELECTRICAL CONTACTS AND METHOD FOR MAKING SAME.

No Drawing.

Application filed October 28, 1918. Serial No. 259,936.

To all whom it may concern:

Be it known that I, FREDERICK L. WHITE, a citizen of the United States, residing at Lakewood, in the county of Cuyahoga and 5 State of Ohio, have invented certain new and useful Improvements in Alloys for Electrical Contacts and Methods for Making Same, of which the following is a specification.

10 This invention relates to alloys, and more particularly to an alloy adapted for contacts for electrical devices.

The main object of the invention is to provide an alloy for electrical contacts, which 15 possesses low resistance, sparks very little, oxidizes but slightly, will retain a smooth and bright contact surface, and will wear well.

Heretofore, it has been thought that a 20 metal or an alloy for electrical contacts should have a high melting point to resist the heat produced by continuous sparking and the dry erosion or wasting away of the contacts as a result thereof. The alloy hereinafter described has been developed on the 25 theory that it is not necessary to use a metal or an alloy having a high melting point, but is more essential that the substance possesses great ductility and malleability.

30 There is great cohesion between the particles of a ductile or malleable substance and consequently when used for electrical contacts, will not flake off in granules as is the case with other substances where there is less cohesion between the particles. As a 35 result, the contacts will wear well, they will remain smooth and bright, there will be but slight sparking, and little oxidization.

The alloy of this invention is produced by 40 treating or reducing compounds of silver in the presence of uranium. To produce an alloy, which when used for electrical contacts has given the best results as herebefore mentioned, silver oxide is reduced in the presence of uranium acetate. The silver oxide

is reduced by adding one-half of one percent of uranium acetate and heating the mixture in a crucible. This alloy when used for electrical contacts, possesses low resistance, and therefore the tendency to become heated is 50 reduced to a minimum with but slight oxidation.

As there is little heat, the effects of spark erosion is lessened, and it is also reduced on account of the great ductility and malleability of the alloy because of the intense cohesion between its particles, which prevents it from flaking off in granules. The contacts therefore wear well, and remain smooth and bright.

It will be understood that this invention consists in producing an alloy by treating or reducing any of the silver salts in the presence of any of the uranium salts.

Having fully described my invention, what I claim is:

1. An alloy for electrical contacts consisting of silver and a sufficient quantity of uranium to increase the cohesion of its particles but less than one per cent of 70 uranium.

2. An alloy for electrical contacts consisting of silver 99½% and uranium ½ of 1%.

3. An alloy for electrical contact points consisting of silver and uranium of a quantity not more than ten percent to prevent it flaking off by electrical action.

4. A method of producing an alloy for electrical contacts consisting of heating a silver oxide and a uranium acetate.

5. A method of producing an alloy for electrical contacts consisting of heating a silver oxide and a sufficient quantity of a uranium acetate to increase the cohesion of its particles but less than one per cent of 85 the uranium acetate.

In testimony whereof I affix my signature.

FREDERICK L. WHITE.